

## UNITED STATES PATENT OFFICE

2,658,317

## PROCESS OF WORKING GLASS

Willard L. Morgan, Pittsburgh, Pa., assignor to  
 Libbey-Owens-Ford Glass Company, Toledo,  
 Ohio, a corporation of Ohio

No Drawing. Application February 23, 1951,  
 Serial No. 212,503

8 Claims. (Cl. 51—283)

1

This invention relates broadly to a process of working glass and is more particularly concerned with the grinding of the edges of the glass or the grinding of surfaces of glass in which some surfaces are being worked upon while others are not.

The invention is further concerned with such operations wherein a cooling fluid, such as water and emulsified oil, is applied to the edging wheels or grinding tools during such work. During such abrading operations, extremely fine particles of glass are continuously removed and these very fine particles are found to be directly soluble to some extent in the water in the cooling fluid. Such solution rapidly becomes alkaline where the fluid is reapplied and reused in a cyclic manner upon the grinding machines. The alkaline solution thus generated is deleterious upon the other surfaces which are not being worked upon and results in etching and loss of finish upon such surfaces.

The invention is also concerned with the processing of completed articles having a glass face such as mirrors and laminated glass. In the case of mirrors where it is desirable to bevel or otherwise finish the edge of the completed mirror having upon one face the mirror film and protective paint backings, it has been found that severe losses due to etching of the uncoated face of the mirror oftentimes results where the mirror edge is being ground by high speed diamond wheels and the cooling lubricant is continuously recycled to such wheels. Likewise, in the grinding of surfaces of optical elements such as prisms, for example, the finishing of successive faces under such circumstances has been found to result in articles which are defective in that the first finished faces are found to be etched due to contact with the fluid during the later treatment of other faces.

In accordance with this invention, it has been found that the above difficulties may be obviated and continuous high speed production machines may be run without encountering such difficulties by the addition of an acid reacting material such as boric acid to the system in which the cooling fluid recirculates. The boric acid reacts with any alkaline condition present in the coolant and reduces the same or creates a slight acid condition, either of which results in cooling fluids which do not etch glass surfaces. Boric acid is particularly effective for this purpose in that, unlike some other acids, it may be added in excessive quantities without any effect upon the glass surfaces or the machines, thus eliminating any requirements as to determining an exact

2

amount to offset the alkalinity present. This is particularly useful since the alkalinity developed in the cooling fluid varies with the amount of glass which has been worked and the total time that the machine has been operated. Thus, it becomes only necessary in the use of boric acid to know that there is an excess of boric acid present in the coolant.

The present invention comprises the additional feature of placing in the cooling fluid a dyestuff or other material which has the properties of changing color in the presence of harmful alkaline conditions. Specifically, the material phenolphthalein is added to the coolant in the form of an alcoholic aqueous solution such as 1% solution in 50% alcohol, and if the solution is harmfully alkaline, it will be indicated to the operator by the solution turning a bright red color. In the presence of excess or free boric acid, the red color from the phenolphthalein is destroyed and the solution becomes colorless. Thus, the operator of the machine is automatically told by the development of the pink color when to add more boric acid to the operation.

Other acids can be employed in place of the boric acid such as hydrochloric or sulfuric acid, but preferably weak acids such as boric acid, oxalic acid, lactic acid, benzoic acid, acetic acid, phthalic acid, phosphoric acid or, more desirably, the acid sodium, potassium, or ammonium phosphates, are used. It is preferred, however, that boric acid or the acid phosphate salts be employed since these are of a nature such that their acidity is so weak that they have no corrosive action upon the machinery when used in excessive amounts, and they further are free of any harmful action upon the skin or clothing of the operators who are subject to contact with the fluid directly during the placement of the work in the machine and its removal therefrom. These last-mentioned materials are also desirable by reason of the fact that they are also solids and the handling of them by the operator is thus very simple. While hazards may thus be involved in the use of the stronger and also liquid acids, it is obvious that these can be employed, and it is merely desirable in such cases that a color changing material be present in the continuously recirculated cooling fluid to signalize to the operator by one color when acid is needed and to signalize by another color when sufficient acid has been added.

Other dyestuffs or so-called indicating materials which may be employed in place of phenolphthalein are methyl red, neutral red, brome

cresol purple, brome thymol blue, and other substances in which a change point comes at a hydrogen ion or pH condition of less than 8.5 and over pH of 4. Preferably, the acidity should never exceed a pH or hydrogen ion condition of 4, since at lower pH's than this the acids will corrode the machinery excessively. Thus, the invention is concerned with maintaining the cooling fluid applied to the glass during the edging, beveling and/or grinding operations within a hydrogen ion or pH condition of less than 8.5 and preferably above 4, and with the inclusion generally in such fluid of an indicating material showing by color changes when the fluid becomes more alkaline than the upper pH of 8.5.

By the use of a combination of phenolphthalein and methyl orange jointly in the circulating fluid, the two dyestuffs will automatically indicate the holding of the acid or alkaline conditions within the range of pH 4 to 8.5 by color changes. Thus, if the pH exceeds 8.5, the solution would be red or pinkish due to the phenolphthalein. In the range of 4 to 8.5, the solution would have a slight yellow tint due to the methyl orange and due to the fact that the phenolphthalein is colorless in such range. At pH's below 4, the solution again would have a red color, but this time due to the fact that the methyl orange produces such red while the phenolphthalein is still colorless. Such a combination of indicators in the circulating fluid would permit the use and addition of any acid material to secure and maintain the solution within this desired range. Specifically, using methyl red as a single indicator, this material is known to change from a red to a yellow when the hydrogen ion condition begins to exceed pH 6. With brome cresol purple, the color goes from a yellow to a purple when the solution exceeds a pH of 7, and with the brome thymol blue the solution becomes blue and changes from yellow when the condition of the fluid exceeds pH 7.5. Specifically, however, phenolphthalein or thymol blue which changes from a blue to a yellow at pH 8.5 are, generally speaking, the preferred indicators where the acids herein provided are employed and particularly where boric acid or the acid sodium phosphates such as monosodium or disodium hydrogen phosphate are used.

In the continuous use of high speed edging, beveling and grinding machines in which the coolant fluid is recirculated, a very considerable amount of finely divided glass is produced which has an extreme amount of surface. From such fine glass material, there is a direct solution out of the same and into the aqueous coolant of alkali as sodium hydroxide and calcium hydroxide, and also a solution of alkali and silica as sodium silicates. These dissolved sodium silicates as well as the alkaline hydroxides are strong alkaline materials. This can be directly demonstrated by mixing powdered glass into water and very quickly it will be found that the solution becomes strongly alkaline. Thus, within twenty minutes after adding such powdered glass to water which was neutral, namely, of a pH or hydrogen ion condition of 7, the alkalinity was found to be 9.1, and after twenty-four hours the alkalinity was found to be pH 11.1. On pouring off such water and repeated by leaching such glass with further additions of water, it will be found that alkali continuously dissolves away from the glass. Even after ten washings, when the glass is left twenty-four hours each time in the water, the pH will be found to rise to 10.2 to 11.1.

The following table gives data on the successive repeated washings with equal quantities of water of the same sample of powdered glass:

| 5  | Number of Washes | Hours of Standing | pH    |
|----|------------------|-------------------|-------|
| 1  |                  | 24                | 11.06 |
| 2  |                  | 24                | 10.48 |
| 3  |                  | 72                | 10.75 |
| 4  |                  | 24                | 8.4   |
| 5  |                  | 24                | 8.2   |
| 6  |                  | 54                | 8.55  |
| 7  |                  | 24                | 8.45  |
| 8  |                  | 24                | 8.45  |
| 9  |                  | 30                | 10.42 |
| 10 |                  | 24                | 10.21 |

The results are typical and the pH's might be higher if a large ratio of powdered glass to water were employed. It clearly shows, however, that alkali dissolves from the glass and, secondly, that alkali continuously dissolves away from the glass even over long periods of time. Such solutions prepared by dissolving powdered glass in water have been found to directly etch glass surfaces when applied to the same and when these are of a pH of over 8.5.

A coolant employed in edging glass that was formed by adding 1 ounce of a self-emulsifying mineral oil to a gallon of water was found to have a pH, when mixed, of 7.9. When this was 30 charged into a clean glass grinding machine used for beveling glass where it was continuously recirculated, the fluid was found to have changed very quickly after the beveling of only twenty 35 rear view automobile mirrors to a pH of 8.96. This was after beveling only 760 lineal inches, and after four such machines had been run for four hours continuously, the coolant was found to be in an alkaline condition in each of a pH of 9.3, 9.9, 10.0, and 10.7, respectively. After running these machines for two weeks, the pH values were up to 10.2, 10.4, 10.6, and 11.1, respectively.

These strongly alkaline solutions as taken from the circulating machines were found to etch the exposed uncoated surface of the mirrors or of 45 glass plates to which such solution was applied. The strongly alkaline solutions were also irritating to the skin of the workers and ate through various types of paint applied to the mirror back, causing additional rejections due to such action 50 through the paint and destroying the silver film. Spoilages of ten to twenty percent under such 55 conditions in the working of rear view automobile mirrors were commonly experienced and have been avoided by the methods of this invention.

Under continuous use of such beveling machines, a very large amount of very finely ground glass accumulates in the circulating system and in particular settles out in the supply tanks 60 and other parts of the machine where the fluid motion is not rapid. This heavy sludge of finely divided glass settles in a very hard and compact mass and approaches a cement-like hard form after a few days use which is extremely difficult 65 to remove from the machinery. Apparently the slow solution of alkali from the surface of the glass causes some sort of reaction with adjacent glass particles resulting in a cementing of the same together, probably through the local formation of a heavy concentration of alkali silicates.

One of the other advantages of the invention is that when the circulating cooling fluid is maintained within a pH range of less than 8.5 and particularly where boric acid is employed, the 75 sludge does not settle into a hard mass but, in-

stead, settles in a very soft dispersed condition which permits easy flushing of the sludge from the machinery. This results in very large savings in maintenance and cleaning of the machines.

By way of contrast to the figures given above which show the development of alkali when continuously beveling glass with a recirculated cooling fluid, the following data shows how, by the use of phenolphthalein indicator and boric acid in the beveling solution, the hydrogen ion condition was kept well within the desired range of less than 8.5.

More specifically, the coolant fluid comprised a solution of 1 gallon of water, 1 ounce of self-emulsifiable mineral oil,  $\frac{1}{15}$  ounce of a one percent phenolphthalein solution in fifty percent alcohol. To the machine, 1 pound of boric acid was added after the zero time reading was made. In the following table it is apparent that the machine was operating under a strongly alkaline condition before the boric acid was added as shown at zero time, and under such condition the solution was bright red due to the phenolphthalein, indicating the presence of such alkali. When the boric acid was added, the solution progressively and quickly lost the red color through gradual shades of pink and became colorless within a few minutes. It will be seen that after one-half hour, the machine was operating in a satisfactory pH range of 7.95 and that this was readily maintained over an extended period by the use of boric acid.

| Time in Hours After Adding Boric Acid | pH                |
|---------------------------------------|-------------------|
| 0.                                    | <sup>1</sup> 10.2 |
| .5.                                   | <sup>2</sup> 7.95 |
| 1.5.                                  | 7.95              |
| 2.5.                                  | 8.00              |
| 3.5.                                  | 8.10              |
| 4.5.                                  | 8.20              |
| 6.5.                                  | 8.20              |
| 24.0.                                 | 7.7               |
| 52.0.                                 | 7.95              |

<sup>1</sup> Acid not added.

<sup>2</sup> Acid added.

In the running of this test, 1 pound of boric acid was added at the end of each twenty-four hours, and the machine was beveling approximately 60,000 lineal inches per day. In such trial where there had been a loss of approximately nine percent of mirrors processed in the machine before the addition of the boric acid, the rejections due to etching of the face of the mirrors and due to spoilage of the mirror film by alkali attack through the protective paint backings were completely eliminated after the boric acid was added to the machine.

In a similar manner where glass prisms were being surfaced using a cooling fluid comprising mostly water and a small amount of emulsified mineral oil, and in which the two finished faces of the prisms were exposed to the coolant during the grinding of the third face, it was found that by the addition of phenolphthalein indicator and boric acid to the circulating fluid system, the rejections due to attack on the glass faces and etching of the same by the circulating fluid were eliminated.

In these operations, boric acid, due to its solid nature, showed to very excellent advantage, resulted in no complaints from the operating personnel, and offered the further advantage that the exact quantity to be added at any time did not have to be predetermined but that any amount might be added to the system provided sufficient was added to destroy any red or pink color and

thereby bring the pH within the desired range of less than 8.5. As boric acid is a material of relatively low water solubility, it has the further advantage that excessive amounts may be added right into the system and the solution of such into the cooling fluid occurs slowly and as needed to offset the alkali being developed by the solution of the glass. Thus, in a sense the limited solubility of boric acid acts to advantage in providing a simple supply mechanism within the fluid. Consequently, no special control is needed in the application of the invention and any unskilled workman can be relied upon to perform the method satisfactorily.

As the above table will indicate, the pH in the system employing boric acid does not fall down within an acid range to any large degree, and it will be recognized that a further function which makes the use of weak acids desirable is that such weak acids, after they react with the alkali present, set up what are known as buffer conditions. That is, the range of pH of the mixture of boric acid and of alkali borate formed by reaction with the alkali falls within fairly narrow ranges, and it is for this reason that the range of pH's shown in the above table of data taken upon the machines falls within the narrow range of pH 7.7 to 8.2. This buffering mechanism functions excellently to permit long time continuous use of the beveling or grinding machines without re-cleaning, since the more sodium borate which is formed, the more the buffering action becomes apparent. Thus, it has become possible to run such machines continuously for several weeks, the only limiting factor being the accumulation of total ground off glass.

It will also be apparent that where a salt of a weak acid such as sodium borate or a sodium phosphate is added to a circulating cooling fluid and an indicating material is also added, the weak acid may be generated right within the coolant by the subsequent addition of another or stronger acid. Thus, the advantages of employing boric acid could also be secured by the addition of ordinary borax along with phenolphthalein and the addition to the solution, whenever it became too alkaline as shown by red color development, of a strong acid such as hydrochloric or phosphoric acids, for example. These strong acids would liberate boric acid within the solution and thereby secure the benefits directly attainable by the use of such. It is obvious of course also that the use of weakly alkaline and weakly acid salt combinations or buffer mixtures may be employed as the source of acidity to be added to the circulating fluid, the proper conditions in any case being indicated through the use of an indicator in the circulating fluid. The invention thus comprises maintaining the circulating fluid within a pH range of less than 8.5 and preferably of over 4 as signalized and indicated by the presence of color changing substances in the fluid and the addition to the fluid of an acid reacting material or other substances which will keep the pH below the desired 8.5. It is apparent that the invention may also be practiced by adding the acids or acid reacting substance to the coolant while maintaining the pH in the desired range of 4 to 8.5 by tests made upon samples of coolant which might be taken from the circulating system. These tests might be made with the indicator color changing materials, or papers containing such, or by well known electrical hydrogen ion or pH determining instruments.

It will be apparent that the acids function to destroy the sodium hydroxide, the calcium hydroxide, and the corresponding alkali silicates which dissolve from the finely ground glass particles by reacting with the same and forming the corresponding alkali salts of such acids. Thus, when boric acid is employed, the sodium hydroxide and silicates would be changed to sodium borate and if hydrochloric acid were used, then sodium chloride would be formed. It is apparent from the well known buffering actions of salts of weak acids that the weak acids offer advantages over the use of the stronger acids. It is also obvious that acids of an organic nature may be employed, such as oxalic, benzoic, and phthalic acids. With the exception of higher cost, the last two offer many of the advantages found with boric acid.

I claim:

1. In the process of working glass, the steps of removing small particles of glass from the main body, applying and recirculating a fluid aqueous cooling media to the area of working during the removal of said particles, and adding an acid reacting material to said cooling media in sufficient quantity to maintain the pH of a solution of the glass particles in the cooling media at a value of less than 8.5 and over 4.

2. In the process of working glass, the steps of removing small particles of glass from the main body of the glass, applying and recirculating a fluid aqueous cooling media in which said particles are soluble to the area of working during the removal of said particles, and adding an acid reacting material to the solution of glass particles and cooling media in sufficient quantity to maintain the pH of said solution at a value of less than 8.5 and over 4.

3. In the process of working glass, the steps of removing small particles of glass from the main body, applying and recirculating a fluid aqueous cooling media to the area of working during the removal of said particles, adding to the cooling media an indicating material characterized by a visual change in color when the pH exceeds 8.5 or is less than 4, and further adding an acid reacting material to said cooling media in sufficient quantity to maintain the pH of a solution of the glass particles in the cooling media within said range.

4. In the process of working glass, the steps of removing small particles of glass from the main body thereof, applying and recirculating a

5 solution of aqueous cooling media comprising an acid reacting material to the area of working during the removal of said particles, and adding said acid reacting material to said solution in sufficient quantity to maintain the pH thereof at a value not exceeding 8.5.

10 5. In the process of working glass, the steps of removing small particles of glass from the main body thereof, applying and recirculating a 10 solution of fluid aqueous cooling media comprising an acid reacting material and a color changing material characterized by a visual change in color when the pH exceeds 8.5 or is less than 4 to the area of working during the removal of said 15 particles, and adding said acid reacting material to said solution in sufficient quantity to maintain the pH thereof within said range.

15 6. In the process of working glass, the steps of removing small particles of glass from the main body thereof, applying a fluid cooling media including a color changing material characterized by a visual change in color when the pH exceeds 8.5 to the main glass body during the removal of said particles, and adding boric acid to a solution 20 of the glass particles in the cooling media when the pH of said solution is observed to exceed 8.5.

25 7. In the process of working glass, the steps of removing small particles of glass from the main body thereof, applying and recirculating a fluid cooling media including a color changing material characterized by a visual change in color when the pH exceeds 8.5 to the main glass body during the removal of said particles, and adding boric acid to a solution 30 of the glass particles in the cooling media when the pH of said solution is observed to exceed 8.5.

35 8. In the process of working glass, the steps of removing small particles of glass from the main body and applying and recirculating to the main glass body during the removal of said particles an aqueous coolant comprising boric acid and an indicating material indicative by a color change of the presence of boric acid in free unreacted form.

45 WILLARD L. MORGAN.

References Cited in the file of this patent

UNITED STATES PATENTS

| Number    | Name   | Date          |
|-----------|--------|---------------|
| 2,366,825 | Adams  | Jan. 9, 1945  |
| 2,387,142 | Fruth  | Oct. 16, 1945 |
| 2,390,405 | Walker | Dec. 4, 1945  |